

# UNITED STATES PATENT OFFICE.

BASIL E. WISE, OF CANTON, OHIO.

## COMPOSITION FOR RAZOR OR OTHER STROPS.

1,353,979.

Specification of Letters Patent. Patented Sept. 28, 1920.

No Drawing.

Application filed August 4, 1919. Serial No. 315,245.

*To all whom it may concern:*

Be it known that I, BASIL E. WISE, a citizen of the United States, residing at Canton, in the county of Stark and State of Ohio, 5 have invented a new and useful Composition for Razor or other Strops, of which the following is a specification.

This invention relates to a new and useful composition to be applied to prepared surfaces such as razor strops or razor stropping devices for the purpose of increasing their efficiency during the honing or stropping of razors, safety razor blades or other sharp instruments; and at the same time imparting pliability to the strop or stropping device to which the composition is applied.

The objects of the invention are to produce a composition of this character which may be easily and readily applied to the 20 surface of a razor strop or stropping device for the purpose of stropping or honing razors, safety razor blades or other sharp edged instruments and at the same time impart pliability to the strop or stropping device to which the composition is applied.

With these objects in view the invention consists in the novel proportions and arrangement of parts, hereinafter described, and particularly pointed out in the appended 30 claims, it being understood that various changes in the form, proportions, and minor details of the composition may be made within the scope of the appended claims, without departing from the spirit or sacrificing any of the advantages of the invention.

My improved composition consists substantially of a mixture of powdered mineral filler of superior quality, such as powdered or pulverized carborundum and aloxite and 40 of superior quality non-poisonous powdered mineral matter, such as talc either white or colored.

In preparing the composition I prefer to use the ingredients in about the following 45 proportions:

8 parts of powdered or pulverized carborundum,

2 parts powdered or pulverized talc; either white or colored.

50 The above ingredients are thoroughly mixed and may be applied as a powder to the surface of the strop or stropping device and when used in the powdered form it may be necessary to add a few drops of fine oil to 55 the surface of the strop or stropping device before applying the composition. It will

be understood that the proportion of the colored talc may be increased should a more pronounced color be desired in the composition. 60

The following formula may also be used in powdered form:

4 parts of powdered or pulverized carborundum,

4 parts powdered or pulverized aloxite, 65

2 parts powdered or pulverized talc, either white or colored.

In preparing the powdered ingredients a very fine sifting device is used to collect any small particles not powdered so that the 70 mixture may be uniform and softened to the proper degree of fineness in order that it may be applied to the most delicate sharp edged instruments.

The composition may also be prepared in 75 paste or cream form with the addition of refined petrolatum to the above named ingredients. It is preferable in preparing the paste or cream to use the following proportions:

8 parts of powdered or pulverized carborundum and aloxite;

2 parts of powdered or pulverized talc, either white or colored;

8 parts of refined petrolatum. 80

The above formula is mixed to a proper consistency ready for immediate use and should be applied in a light coat upon the strop or stropping device and smoothed with the palm of the hand. Good results may 90 also be obtained when all of the minerals are blended with parowax in the following proportions:

4 parts powdered or pulverized carborundum; 95

4 parts powdered or pulverized aloxite;

2 parts powdered or pulverized talc; either white or colored;

5 parts parowax.

The powdered minerals when properly blended are then added to the parowax which has been reduced to a liquid form and the composition is then mixed to a proper consistency and placed in earthen or metal molds of a desired shape or in wooden forms and allowed to cool to a solid state when it is ready for use. 100

The powdered or pulverized minerals entering into this composition should be the finest that can be obtained in the market. 110 The powdered talc is used in the composition as a medium to reduce the ingredients

to a variable powdered consistency, and can be more readily used in a dusting or sifting process and lends a mellowed softness to the composition which may be applied to the 5 most delicate sharp edged instruments with satisfactory results. The petrolatum is used to reduce the powdered ingredients to the cream or paste form and the parowax to reduce the powdered ingredients to solid form 10 or to any desired consistency which may be obtained by varying the proportions of the different ingredients and which will yet be susceptible to sharp edged instruments for honing and stropping purposes.

15 The composition is not restricted to the exact proportions of the different ingredients as above set forth as these proportions may be more or less varied as requirements and conditions of the ingredients used may 20 call for a variation in the proportions used. This composition may not only serve to constitute an abrading surface of superior quality for honing or stropping razors, safety razor blades and the like but it will 25 also serve to preserve the necessary pliability and suppleness of the strop or other surface to which it is applied.

Although the above specification discloses the best mode in which I have contemplated embodying my invention I desire 30 to be not limited to the details of such disclosure, for, in the further practical application of my invention many changes in form, construction and proportions may be made 35 as circumstances require or experience suggests, without departing from the spirit of the invention within the scope of the appended claims.

I claim:

1. A composition for razor strops or the 40 like for honing purposes composed of powdered or pulverized carborundum, powdered or pulverized aloxite, powdered talc and petrolatum and parowax.
2. A composition for razor strops or the 45 like for honing purposes, comprising about four parts of powdered or pulverized carborundum, four parts of powdered or pulverized aloxite, two parts of powdered talc and eight parts of petrolatum to be used in 50 cream or paste form.

In testimony that I claim the above, I have hereunto subscribed my name.

BASIL E. WISE.